

Patented Oct. 30, 1928.

1,689,426

# UNITED STATES PATENT OFFICE.

CAMILLE DREYFUS, OF NEW YORK, N. Y., AND HERBERT PLATT, OF CUMBERLAND, MARYLAND, ASSIGNORS TO CELANESE CORPORATION OF AMERICA, A CORPORATION OF DELAWARE.

## DIFFERENTIAL COLORED FABRIC AND METHOD OF MAKING SAME.

No Drawing.

Application filed August 13, 1927. Serial No. 212,832.

This invention relates to fabric having a design thereon which design is due to the difference of the effects of dyes upon the material of which the fabric is composed and 5 the material with which the fabric is printed.

An object of our invention is to provide a fabric having a design thereon, which design is not made by the ordinary process of printing by means of dyes or other colors, but 10 which is obtained by the differential dyeing of the fabric due to the printing or the application by other means of material upon such fabric, which material is affected by dyes in a manner different from the material 15 of which the fabric is composed.

Another object of our invention is to provide a fabric which is cross-dyed, wherein color effect or design produced is independent of the weave but which may be produced in any desired configuration.

Another object of our invention is to produce a design by cross-dyeing upon a fabric composed at least in part of an organic derivative of cellulose having a design of 20 cellulose printed thereon.

Other objects of our invention will appear from the following detailed description.

It is well known that cellulose, whether natural cellulose such as cotton, or reconstituted cellulose such as is obtained from viscose, reacts in a different manner from cellulose acetate silk, natural silk or wool towards many dyes, or that differential effects may be obtained by dyeing a mixture 30 of cellulose and these fibres in one bath containing a dye or mixture of dyes. This principle is used commonly in cross-dyeing mixed fabrics made by weaving yarns of cotton and one of the above mentioned materials. Obviously in this method, the differential color effect depends entirely upon 40 the nature of the weave. In accordance with our invention, cross-dyeing effects are obtained by making a design of cellulose, irrespective of weaving, on a fabric which contains at least some yarn of a material other than cellulose, and then immersing the 45 fabric in a bath containing one or more dyes having different coloring effects upon the cotton and the other material.

The fabric to be treated may be made entirely of an organic derivative of cellulose, such as organic esters of cellulose or organic ethers of cellulose. Examples of organic

esters of cellulose that may be used are 55 cellulose formate, cellulose acetate, cellulose propionate and cellulose butyrate. Examples of cellulose ethers that may be used are methyl cellulose and ethyl cellulose. Or the fabric may be composed of a mixture 60 of any of the above organic derivatives of cellulose with one or more other fibres such as natural silk, wool, cotton or reconstituted cellulose. Furthermore the fabric to be treated may be composed wholly of silk or 65 wool or a mixture of these animal fibres.

The fabric, constituted as above set forth, is printed with a material whose behavior toward dyestuffs is different from that of organic derivative of cellulose, natural silk 70 or wool. Among the materials used for this purpose may be mentioned cellulose, gelatin or casein. The so printed fabric is then dyed in a differential dye bath.

One mode of carrying out our invention 75 is to print the fabric, constituted as above set forth, with one of the common solutions of cellulose used in making reconstituted cellulose artificial silk, such as a solution of cellulose xanthate (viscose) or a cuprammonium solution of cellulose. The thickness or concentration of the cellulose solution to be used for printing may be varied in accordance with the type of fabric to be treated or the nature of the design desired. 80

After the fabric has been printed with the cellulose solution, it is permitted to dry if desired. The fabric is then treated to re-convert the cellulose compound of the print back to cellulose. For instance, if viscose 90 has been used for printing, the cellulose is reconstituted by immersing the fabric in a dilute aqueous solution of sulphuric acid. Better results may be obtained by using a solution of sodium acid sulfate, or a solution of sodium acid sulfate and sodium sulfate as the precipitating bath. The fabric now has a design of cellulose imprinted or impressed upon it. The fabric may now 95 be washed and/or dried if desired. It is 100 now ready for the dyeing treatment.

The fabric, which contains at least some fibres or yarns of one or more of the following substances, viz, organic derivative of cellulose, silk, wool, or some other fibre other than cellulose, and which has a design of cellulose imprinted thereon, is now placed 105 in a dye bath which contains one or more

dyes which act differently towards the cellulose and the other material of which at least some of the fibres are composed. Thus the dye may color cellulose and not color the other material, or it may color the cellulose more deeply than the other material. On the other hand the dye may color the other material and not color the cellulose or else color the other material more deeply than the cellulose. Again, the dye bath may contain two or more dyes, one of which colors the other material and not the cellulose, while the other of which colors the cellulose but not the other material. When using such mixtures of dyes, it will be seen that by immersion of the fabric so printed with cellulose in a single dye bath, a two-colored design may be produced. The fabric is then given the ordinary finishing treatment.

When the fabric treated according to the above process is made of mixed yarns containing cotton, such as mixed cellulose acetate and cotton, mixed natural silk and cotton, or mixed wool and cotton, the cotton yarn will be dyed or remain undyed in the same manner as the cellulose of the print. This will give the double effect of ordinary cross-dyeing of mixed fabrics together with the effect of the cross-dyeing of the printed cellulose design.

In another application of our invention, the fabric constituted as above set forth, is printed with a solution of gelatin or a solution of casein, and then dyed. The parts of the fabric printed by the gelatin or casein are not affected by the dyes and thus differential color effects are obtained. The gelatin or casein is then washed off by appropriate treatment and the fabric is then finished in any appropriate manner.

To further elucidate the mode of carrying out our invention, the following specific examples are given by way of illustration only:

#### Example I.

A tricot knit fabric made of cellulose acetate is printed with a solution of viscose (sodium xanthate) and the cellulose is then precipitated by means of a dilute solution of sulphuric acid. The fabric now consists of cellulose acetate yarn having a design of a cellulose printed thereon. It is now immersed in a 30-1 dye bath containing a dye which dyes cellulose acetate blue and which does not affect cellulose and a dye which dyes cellulose yellow and which does not affect the cellulose acetate. This dye bath is made up as follows:

|                                                                | Per cent. |
|----------------------------------------------------------------|-----------|
| SRA blue IV                                                    | 0.5       |
| CR cotton fast yellow B (color index #842 Schultz-Julius #617) | 1.0       |
| Glauber's salt (sodium sulfate)                                | 30        |

The percentages given are based on the weight of the fabric treated.

After finishing in the ordinary manner the background of the fabric is colored blue, while the design is of a greenish color due to the combined effects of the yellow color of the cellulose print and the blue of the cellulose fabric under the print.

#### Example II.

A tricot knit cellulose acetate fabric is printed with cellulose in the manner set forth in Example I. It is now immersed in a dye bath containing a dye which dyes cellulose acetate fibre blue and which does not affect cellulose and a dye which dyes cellulose red and which does not affect cellulose acetate. This dye bath is made up as follows:

|                                                                    | Per cent. |
|--------------------------------------------------------------------|-----------|
| SRA blue IV                                                        | 0.5       |
| CR cotton fast scarlet 4 BS (color index #327 Schultz-Julius #279) | 0.5       |
| Glauber's salt                                                     | 30        |

The percentages given are based on the weight of the fabric treated.

After finishing in the ordinary manner the background of the fabric is colored blue while the design is of a greyish-purple due to the combination of the red color of the cellulose acetate print and the blue color of the cellulose acetate fabric under the print.

#### Example III.

A cellulose acetate satin is printed with cellulose in the manner set forth in Example I. It is then immersed in a dye bath containing a dye which dyes cellulose brown but which does not affect the cellulose acetate. This dye bath is made up as follows:

|                                           | Per cent. |
|-------------------------------------------|-----------|
| CR cotton fast brown R (color index #597) | 0.5       |
| Glauber's salt                            | 30        |

The percentages given are based on the weight of the fabric treated.

After finishing in the ordinary manner the background of the fabric is of the original natural color of the cellulose acetate silk (white) while the design is brown.

#### Example IV.

A tricot knit cellulose acetate fabric is printed with cellulose in the manner set forth in Example I. It is now immersed in a dye bath containing a dye which colors cellulose red but which does not affect the cellulose acetate silk. This dye bath is made up as follows:

|                        | Per cent. |
|------------------------|-----------|
| CR cotton scarlet 4 BS | 0.5       |
| Glauber's salt         | 30        |

The percentages given are based on the weight of the fabric treated.

After finishing in the ordinary manner the background of the fabric is of the original natural color of the cellulose acetate (white) while the design is red.

5 The foregoing examples are given merely by way of illustration of modes of carrying out our invention. It is to be understood that many variations may be made therein without departing from the spirit of the invention. Instead of cellulose acetate, organic derivatives of cellulose may be used such as cellulose esters, e. g. cellulose formate, cellulose propionate or cellulose butyrate, or cellulose ethers e. g. methyl cellulose 10 or ethyl cellulose.

Having described our invention what we claim and desire to secure by Letters Patent is:—

20 1. A fabric comprising yarn of a material other than cellulose having a design of cellulose material imprinted thereon.

25 2. A fabric comprising yarn of an organic derivative of cellulose material having a design of cellulose material imprinted thereon.

30 3. A fabric comprising yarn of cellulose acetate material having a design of cellulose material imprinted thereon.

35 4. A fabric comprising yarn of a material other than cellulose having a design of cellulose material imprinted thereon said yarn having a color different from said design of cellulose.

40 5. A fabric comprising yarn of an organic derivative of cellulose material having a design imprinted thereon said yarn having a color different from said design of cellulose.

45 6. A fabric comprising yarn of cellulose acetate material having a design of cellulose material imprinted thereon said yarn having a color different from said design of cellulose.

50 7. A fabric comprising yarn of a material other than cellulose having a design of cellulose material imprinted thereon at least one of said materials being dyed by a dye that does not impart color to the other material.

55 8. A fabric comprising yarn of cellulose acetate material having a design of cellulose material imprinted thereon at least one of said materials being dyed by a dye that does not impart color to the other material.

60 9. A fabric comprising yarn of an organic derivative of cellulose material having a design of cellulose material imprinted thereon said organic derivative of cellulose material being dyed by a dye which does not substantially color the cellulose and said cellulose being dyed by a dye which does not substantially color said organic derivative of cellulose.

65 10. A fabric comprising yarn of cellulose acetate material having a design of cellulose material imprinted thereon said cellulose

acetate material being dyed by a dye which does not substantially color the cellulose and said cellulose being dyed by a dye which does not appreciably color said cellulose acetate.

11. A process which comprises imprinting 70 a design of a solution of cellulose material on a fabric comprising yarn of a material other than cellulose and treating the so printed fabric with a solution adapted to reconstitute the cellulose material of the print.

12. A process which comprises imprinting 75 a design of a solution of cellulose material on a fabric comprising yarn of an organic derivative of cellulose material and treating the so printed fabric with a solution adapted 80 to reconstitute the cellulose material of the print.

13. A process which comprises imprinting 85 a design of a solution of cellulose material on a fabric comprising yarn of cellulose acetate material and treating the so printed fabric with a solution adapted to reconstitute the cellulose material of the print.

14. A process which comprises imprinting 90 a design of a solution of cellulose material on a fabric comprising yarn of an organic derivative of cellulose material, treating the so printed fabric with a solution adapted to reconstitute the cellulose material of the print and dyeing with a dye that does not 95 dye said cellulose and said organic derivative of cellulose the same shade.

15. A process which comprises imprinting 100 a design of a solution of cellulose material on a fabric comprising yarn of cellulose acetate, treating the so printed fabric with a solution adapted to reconstitute the cellulose material of the print and dyeing with a dye that does not dye said cellulose and said cellulose acetate the same shade.

16. A process which comprises imprinting 110 a design of a solution of cellulose material on a fabric comprising yarn of an organic derivative of cellulose, treating the so printed fabric with a solution adapted to reconstitute the cellulose material of the print, and treating the fabric with a dye which colors one of the said materials but does not appreciably color the other material.

17. A process which comprises imprinting 115 a design of a solution of cellulose material on a fabric comprising yarn of cellulose acetate, treating the so printed fabric with a solution adapted to reconstitute the cellulose material of the print and treating the fabric with a dye which colors one of the said materials but does not appreciably color the other material.

18. A process which comprises imprinting 125 a design of a solution of cellulose material on a fabric comprising yarn of an organic derivative of cellulose material, treating the so printed fabric with a solution adapted to reconstitute the cellulose material of the print and treating in a bath containing a dye 130

which dyes said organic derivative of cellulose but does not appreciably color said organic derivative of cellulose.

19. A process which comprises imprinting a design of a solution of cellulose material on a fabric comprising yarn of cellulose acetate material, treating the so printed fabric with a solution adapted to reconstitute the cellulose material of the print and treating

in a bath containing a dye which dyes said 10 cellulose acetate but does not substantially color said cellulose and a dye which dyes the cellulose but does not substantially color said cellulose acetate.

In testimony whereof, they have hereunto 15 subscribed their names.

CAMILLE DREYFUS.  
HERBERT PLATT.